



US007462433B2

(12) **United States Patent**  
**Wu et al.**

(10) **Patent No.:** **US 7,462,433 B2**  
(45) **Date of Patent:** **\*Dec. 9, 2008**

(54) **PHOTORECEPTOR ADDITIVE**

(75) Inventors: **Jin Wu**, Webster, NY (US); **Daniel V. Levy**, Rochester, NY (US); **Liang-bih Lin**, Rochester, NY (US); **Marc J. Livecchi**, Rochester, NY (US)

(73) Assignee: **Xerox Corporation**, Norwalk, CT (US)

(\*) Notice: Subject to any disclaimer, the term of this patent is extended or adjusted under 35 U.S.C. 154(b) by 433 days.

This patent is subject to a terminal disclaimer.

(21) Appl. No.: **11/213,522**

(22) Filed: **Aug. 26, 2005**

(65) **Prior Publication Data**

US 2007/0048639 A1 Mar. 1, 2007

(51) **Int. Cl.**

**G03G 15/04** (2006.01)

(52) **U.S. Cl.** ..... **430/60**; 430/64; 430/65;  
430/131

(58) **Field of Classification Search** ..... 430/60,  
430/64, 65, 131

See application file for complete search history.

(56) **References Cited**

## U.S. PATENT DOCUMENTS

|             |         |             |
|-------------|---------|-------------|
| 4,464,450 A | 8/1984  | Teuscher    |
| 4,518,669 A | 5/1985  | Yashiki     |
| 4,579,801 A | 4/1986  | Yashiki     |
| 4,775,605 A | 10/1988 | Seki et al. |

|                   |         |                              |
|-------------------|---------|------------------------------|
| 5,017,449 A       | 5/1991  | Yoshihara                    |
| 5,344,734 A       | 9/1994  | Monbaliu et al.              |
| 5,385,796 A       | 1/1995  | Spiewak et al.               |
| 5,449,573 A       | 9/1995  | Aoki et al.                  |
| 5,489,496 A       | 2/1996  | Katayama et al.              |
| 5,641,599 A       | 6/1997  | Markovics et al.             |
| 5,656,407 A       | 8/1997  | Kawahara                     |
| 5,721,080 A       | 2/1998  | Terrell et al.               |
| 5,928,824 A       | 7/1999  | Obinata et al.               |
| 6,180,309 B1      | 1/2001  | Maty et al.                  |
| 6,200,716 B1      | 3/2001  | Fuller et al.                |
| 6,207,334 B1      | 3/2001  | Dinh et al.                  |
| 6,858,363 B2 *    | 2/2005  | Belknap et al. .... 430/65   |
| 6,946,226 B2 *    | 9/2005  | Wu et al. .... 430/64        |
| 7,153,574 B2 *    | 12/2006 | Qi et al. .... 428/403       |
| 2004/0197686 A1 * | 10/2004 | Belknap et al. .... 430/58.8 |
| 2005/0042533 A1 * | 2/2005  | Wu et al. .... 430/64        |

## OTHER PUBLICATIONS

U.S. Appl. No. 10/942,277, filed Sep. 16, 2004.  
Sorenson et al., *Preparative Methods of Polymer Chemistry*, 2nd ed.,  
Interscience Publishers, pp. 76-77.  
Sorenson et al., *Preparative Methods of Polymer Chemistry*, 2nd ed.,  
Interscience Publishers, pp. 76-77, 1968.

\* cited by examiner

Primary Examiner—Mark A Chapman

(74) Attorney, Agent, or Firm—Pillsbury Winthrop Shaw  
Pittman LLP

(57) **ABSTRACT**

The presently disclosed embodiments relate in general to electrophotographic imaging members, such as layered photoreceptor structures, and processes for making and using the same. More particularly, the embodiments pertain to a photoreceptor additive to improve image quality.

**16 Claims, No Drawings**

## PHOTORECEPTOR ADDITIVE

## BACKGROUND

The invention relates generally to electrophotographic imaging members, such as layered photoreceptor structures, and processes for making and using the same. More particularly, the embodiments pertain to a photoreceptor additive to improve image quality.

Electrophotographic imaging members, e.g., photoreceptors, typically include a photoconductive layer formed on an electrically conductive substrate. The photoconductive layer is an insulator in the substantial absence of light so that electric charges are retained on its surface. Upon exposure to light, the charge is dissipated.

In electrophotography, also known as Xerography, electrophotographic imaging or electrostatographic imaging, the surface of an electrophotographic plate, drum, belt or the like (imaging member or photoreceptor) containing a photoconductive insulating layer on a conductive layer is first uniformly electrostatically charged. The imaging member is then exposed to a pattern of activating electromagnetic radiation, such as light. The radiation selectively dissipates the charge on the illuminated areas of the photoconductive insulating layer while leaving behind an electrostatic latent image. This electrostatic latent image may then be developed to form a visible image by depositing oppositely charged particles on the surface of the photoconductive insulating layer. The resulting visible image may then be transferred from the imaging member directly or indirectly (such as by a transfer or other member) to a print substrate, such as transparency or paper. The imaging process may be repeated many times with reusable imaging members.

An electrophotographic imaging member may be provided in a number of forms. For example, the imaging member may be a homogeneous layer of a single material such as vitreous selenium or it may be a composite layer containing a photoconductor and another material. In addition, the imaging member may be layered. These layers can be in any order, and sometimes can be combined in a single or mixed layer.

The demand for improved print quality in xerographic reproduction is increasing, especially with the advent of color. Common print quality issues are strongly dependent on the quality of the undercoat layer. Conventional materials used for the undercoat or blocking layer have been problematic. In certain situations, a thicker undercoat is desirable, but the thickness of the material used for the undercoat layer is limited by the inefficient transport of the photo-injected electrons from the generator layer to the substrate. If the undercoat layer is too thin, then incomplete coverage of the substrate results due to wetting problems on localized unclean substrate surface areas. The incomplete coverage produces pin holes which can, in turn, produce print defects such as charge deficient spots ("CDS") and bias charge roll ("BCR") leakage breakdown. Other problems include "ghosting," which is thought to result from the accumulation of charge somewhere in the photoreceptor. Consequently, when a sequential image is printed, the accumulated charge results in image density changes in the current printed image that reveals the previously printed image. Thus, there is a need, which the present invention addresses, for a way to minimize or eliminate charge accumulation in photoreceptors, without sacrificing the desired thickness of the undercoat layer.

The terms "charge blocking layer" and "blocking layer" are generally used interchangeably with the phrase "undercoat layer."

Conventional photoreceptors and their materials are disclosed in Katayama et al., U.S. Pat. No. 5,489,496; Yashiki, U.S. Pat. No. 4,579,801; Yashiki, U.S. Pat. No. 4,518,669; Seki et al., U.S. Pat. No. 4,775,605; Kawahara, U.S. Pat. No. 5,656,407; Markovics et al., U.S. Pat. No. 5,641,599; Mombaliu et al., U.S. Pat. No. 5,344,734; Terrell et al., U.S. Pat. No. 5,721,080; and Yoshihara, U.S. Pat. No. 5,017,449, which are herein all incorporated by reference.

More recent photoreceptors are disclosed in Fuller et al., 10 U.S. Pat. No. 6,200,716; Maty et al., U.S. Pat. No. 6,180,309; and Dinh et al., U.S. Pat. No. 6,207,334, which are all herein incorporated by reference.

Conventional undercoat or charge blocking layers are also disclosed in U.S. Pat. No. 4,464,450; U.S. Pat. No. 5,449,573; 15 U.S. Pat. No. 5,385,796; and Obinata et al., U.S. Pat. No. 5,928,824, which are all herein incorporated by reference.

## SUMMARY

20 According to embodiments illustrated herein, there is provided a way in which print quality is improved, for example, ghosting is minimized or substantially eliminated in images printed in systems with high transfer current.

In particular, an embodiment of the present invention provides 25 an electrophotographic imaging member, comprising a substrate, an undercoat layer formed on the substrate, where the undercoat layer comprises a charge transfer molecule/metal oxide complex, and at least one imaging layer formed on the undercoat layer.

30 Embodiments of the present invention also provides processes with which to prepare such an imaging member, comprising forming a coating mixture by blending a dispersion containing  $TiO_2$  with a charge transfer molecule, thereby forming a charge transfer molecule/ $TiO_2$  complex, applying 35 the coating mixture on an electrophotographic imaging member, and causing the coating mixture to form an undercoat layer containing the charge transfer molecule/ $TiO_2$  complex on the electrophotographic imaging member.

In another embodiment, there is described a process for 40 preparing an electrophotographic imaging member, comprising forming a coating mixture by dispersing a formulation containing  $TiO_2$  and a charge transfer molecule, thereby forming a charge transfer molecule/ $TiO_2$  complex, applying the coating mixture on an electrophotographic imaging member, and causing the coating mixture to form an undercoat layer containing the charge transfer molecule/ $TiO_2$  complex on the electrophotographic imaging member.

An alternative embodiment provides for a process for preparing 45 an electrophotographic imaging member, comprising treating the surface of  $TiO_2$  with a charge transfer molecule, thereby forming a charge transfer molecule/ $TiO_2$  complex, dispersing the treated  $TiO_2$ , applying the coating mixture on an electrophotographic imaging member, and causing the coating mixture to form an undercoat layer containing the 50 charge transfer molecule/ $TiO_2$  complex on the electrophotographic imaging member.

## DETAILED DESCRIPTION

60 In the following description, reference is made to the accompanying drawings, which form a part hereof and which illustrate several embodiments of the present invention. It is understood that other embodiments may be utilized and structural and operational changes may be made without departure 65 from the scope of the present invention.

Embodiments of the present invention relate to a photoreceptor having a undercoat layer which incorporates an addi-

tive to the formulation that helps reduce, and preferably substantially eliminates, specific printing defects in the print images.

According to embodiments of the present invention, an electrophotographic imaging member is provided, which generally comprises at least a substrate layer, an undercoat layer, and an imaging layer. The undercoating layer is generally located between the substrate and the imaging layer, although additional layers may be present and located between these layers. The imaging member may also include a charge generating layer and a charge transport layer. This imaging member can be employed in the imaging process of electrophotography, where the surface of an electrophotographic plate, drum, belt or the like (imaging member or photoreceptor) containing a photoconductive insulating layer on a conductive layer is first uniformly electro statically charged. The imaging member is then exposed to a pattern of activating electromagnetic radiation, such as light. The radiation selectively dissipates the charge on the illuminated areas of the photoconductive insulating layer while leaving behind an electrostatic latent image. This electrostatic latent image may then be developed to form a visible image by depositing oppositely charged particles on the surface of the photoconductive insulating layer. The resulting visible image may then be transferred from the imaging member directly or indirectly (such as by a transfer or other member) to a print substrate, such as transparency or paper. The imaging process may be repeated many times with reusable imaging members.

Thick undercoat layers are desirable for photoreceptors due to their life extension and carbon fiber resistance. Furthermore, thicker undercoat layers make it possible to use less costly substrates in the photoreceptors. Such thick undercoat layers have been developed, such as one developed by Xerox Corporation and disclosed in U.S. patent application Ser. No. 10/942,277, filed Sep. 16, 2004, entitled "Photoconductive Imaging Members," which is hereby incorporated by reference. However, due to insufficient electron conductivity in dry and cold environments, the residual potential in conditions known as "J zone" (10% room humidity and 70° F.) is unacceptably high (e.g., >150V) when the undercoat layer is thicker than 15  $\mu$ m.

Common print quality issues are strongly dependent on the quality of the undercoat layer. Conventional materials used for the undercoat or blocking layer have been problematic because print quality issues are strongly dependent on the quality of the undercoat layer. For example, charge deficient spots ("CDS") and bias charge roll ("BCR") leakage breakdown are problems the commonly occur. Another problem is "ghosting," which is thought to result from the accumulation of charge somewhere in the photoreceptor. Consequently, when a sequential image is printed, the accumulated charge results in image density changes in the current printed image that reveals the previously printed image.

There have been formulations developed for undercoat layers that, while suitable for their intended purpose, do not address the ghosting effect problem. To alleviate the problems associated with charge block layer thickness and high transfer currents, the addition of a charge transfer molecule to a formulation containing  $TiO_2$  is performed to help reduce and preferably substantially eliminate ghosting failure in xerographic reproductions. This addition step produces a charge transfer molecule/metal oxide complex that is shown to be useful in reducing ghosting.

In various embodiments, charge transfer molecule can chelate with  $TiO_2$ , and changes its color, thus forming a charge

transfer molecule/ $TiO_2$  complex. A charge transfer molecule consists of one or more sub-structures in its molecule with formula(s) of:



wherein Z is independently selected from the group consisting of a hydroxyl and a thio, X is independently selected from the group consisting of a hydroxyl, a thio, and a halogen atom, and Y is independently selected from the group consisting of an oxygen and a sulfur atom. The halogen atom may be, for example, F, Cl, Br, or I. Examples of charge transfer molecules include, but are not limited to, catechol, 4-methyl-1, 2-benzenediol, 3-methyl-1,2-benzenediol, 1,2,4-benzenetriol, 1,2,3-benzenetriol, 3-fluoro-1,2-benzenediol, 3,4-dihydroxybenzonitrile, 3-methoxy-1,2-benzenediol, 5-methyl-1,2,3-benzenetriol, 2-fluoro-6-methoxyphenol, 4-chloro-1,2-benzenediol, 1,2-naphthalenediol, 2,3-naphthalenediol, 7,8-dihydroxy-2H-chromen-2-one, 6,7-dihydroxy-2H-chromen-2-one, 3,5-dichloro-1,2-benzenediol, 2-hydroxy-3,4-dimethoxybenzaldehyde, 2-chloro-4-(hydroxymethyl)-6-methoxyphenol, 2,3,4,6-tetrahydroxy-5H-benzo[a]cyclohepten-5-one, 1,2,10-anthracenetriol, 1,2-dihydroxyanthra-9,10-quinone (alizarin), 3,4,5,6-tetrachloro-1,2-benzenediol, 7,8-dihydroxy-2-phenyl-4H-chromen-4-one, 1,2,7-trihydroxyanthra-9,10-quinone, 1,2,4-trihydroxyanthra-9,10-quinone, 3,4,5,6-tetrachloro-1,2-benzenediol, 7,8-dihydroxy-2-methyl-3-phenyl-4H-chromen-4-one, 5,6,7-trihydroxy-2-phenyl-4H-chromen-4-one, 1,2,5,8-tetrahydroxyanthra-9,10-quinone (quinalizarin), 2-(3,4-dihydroxyphenyl)-5,7-dihydroxy-4H-chromen-4-one, 3,4,6a,10-tetrahydroxy-6a,7-dihydroindeno[2,1-c]chromen-9(6H)-one, 3,7-dihydroxy-2-(4-hydroxy-3-methoxyphenyl)-4H-chromen-4-one, 2,3,7,8-tetrahydroxychromeno[5,4,3-cde]chromene-5,10-dione, 2-(3,4-dihydroxyphenyl)-3,5,7-trihydroxy-4H-chromen-4-one, nordihydroguaiaretic acid, tetrachlorocatechol, 2,4,5-trichlorophenol, 2,2'-bi(3-hydroxy-1,4-naphthoquinone), tetrahydroxy-1,4-quinone, 8-hydroxyquinoline, 4',5'-dibromo-9-phenyl-2,3,7-trihydroxy-6-fluorone, 1,2,3,4-tetrafluoro-5,8-dihydroxyanthraquinone, and the like and mixtures thereof.

In embodiments,  $TiO_2$  can be either surface treated or untreated. Surface treatments include, but are not limited to aluminum laurate, alumina, zirconia, silica, silane, methicone, dimethicone, sodium metaphosphate, and the like and mixtures thereof. Examples of  $TiO_2$  include MT-150W (surface treatment with sodium metaphosphate, Tayca Corporation), STR-60N (no surface treatment, Sakai Chemical Industry Co., Ltd.), FTL-100 (no surface treatment, Ishihara Sangyo Laisha, Ltd.), STR-60 (surface treatment with  $Al_2O_3$ , Sakai Chemical Industry Co., Ltd.), TTO-55N (no surface treatment, Ishihara Sangyo Laisha, Ltd.), TTO-55A (surface treatment with  $Al_2O_3$ , Ishihara Sangyo Laisha, Ltd.), MT-150AW (no surface treatment, Tayca Corporation), MT-150A (no surface treatment, Tayca Corporation), MT-100S (surface treatment with aluminum laurate and alumina, Tayca Corporation), MT-100HD (surface treatment with zirconia and alumina, Tayca Corporation), MT-100SA (surface treatment with silica and alumina, Tayca Corporation), and the like.

Undercoat layer binder materials are well known in the art. Typical undercoat layer binder materials include, for example, polyesters, MOR-ESTER 49,000 from Morton International Inc., VITEL PE-100, VITEL PE-200, VITEL PE-200D, and VITEL PE-222 from Goodyear Tire and Rubber Co., polyarylates such as ARDEL from AMOCO Production Products, polysulfone from AMOCO Production Products, polyurethanes, and the like. Other examples of suitable undercoat layer binder materials include, but are not limited to, a polyamide such as Luckamide 5003 from DAINIPPON Ink and Chemicals, Nylon 8 with methylmethoxy pendant groups, CM 4000 and CM 8000 from Toray Industries Ltd and other N-methoxymethylated polyamides, such as those prepared according to the method described in Sorenson and Campbell "Preparative Methods of Polymer Chemistry" second edition, p. 76, John Wiley and Sons Inc. (1968), and the like and mixtures thereof. These polyamides can be alcohol soluble, for example, with polar functional groups, such as methoxy, ethoxy and hydroxy groups, pendant from the polymer backbone. Another examples of undercoat layer binder materials include phenolic-formaldehyde resin such as VARCUM 29159 from OXYCHEM, aminoplast-formaldehyde resin such as CYMEL resins from CYTEC, poly (vinyl butyral) such as BM-1 from Sekisui Chemical, and the like and mixtures thereof.

The weight/weight ratio of charge transfer molecule and  $TiO_2$  in the charge transfer molecule/ $TiO_2$  complex is from about 0.0001/1 to about 0.2/1, or from about 0.001/1 to about 0.05/1, or from about 0.005/1 to about 0.02/1.

The undercoat layer consists of the above charge transfer molecule/ $TiO_2$  complex and polymeric binder. The weight/weight ratio of the charge transfer molecule/ $TiO_2$  complex and the binder is from about 20/80 to about 80/20, or from about 40/60 to about 65/35.

In various embodiments, the undercoat layer further contains an optional light scattering particle. In various embodiments, the light scattering particle has a refractive index different from the binder and has a number average particle size greater than about 0.8  $\mu m$ . The light scattering particle can be amorphous silica or silicone ball. In various embodiments, the light scattering particle can be present in an amount of from about 0% to about 10% by weight of the total weight of the undercoat layer.

In various embodiments, the undercoat layer has a thickness of from about 0.1  $\mu m$  to about 30  $\mu m$ , or from about 2  $\mu m$  to about 25  $\mu m$ , or from about 10  $\mu m$  to about 20  $\mu m$ . In further embodiments, the charge transfer molecule/metal oxide complex is present in an amount of from about 20% to about 80%, or from about 40% to about 65%, by weight of the total weight of the undercoat layer. In still further embodiments, the charge transfer molecule is present in an amount of from about 0.1% to about 5%, or from 0.5% to about 2%, by weight of the charge transfer molecule/metal oxide complex.

In various embodiments, the charge transfer molecule is 2,2'-bi(3-hydroxy-1,4-naphthoquinone). There are three methods with which to incorporate the additive into the formulation: (1) the first involves simple mixing of 2,2'-bi(3-hydroxy-1,4-naphthoquinone) with a dispersion of  $TiO_2$  MT-150W, phenolic resin VARCUM 29159, melamine resin CYMEL 323 in xylene, 1-butanol, and methyl ethyl ketone (MEK) with the dispersion being prepared beforehand via ball milling; (2) the second involves ball milling 2,2'-bi(3-hydroxy-1,4-naphthoquinone) with the formulation of  $TiO_2$  MT-150W, phenolic resin VARCUM 29159, melamine resin CYMEL 323 in xylene, 1-butanol, and MEK; and (3) the third involves treating the surface of  $TiO_2$  MT-150W with 2,2'-bi(3-hydroxy-1,4-naphthoquinone) first, followed by ball mill-

ing the 2,2'-bi(3-hydroxy-1,4-naphthoquinone)/ $TiO_2$  MT-150W charge transfer complex, phenolic resin VARCUM 29159, melamine resin CYMEL 323 in xylene, 1-butanol, and MEK. The  $TiO_2$  may have a powder volume resistivity of from about  $1 \times 10^4$  to about  $1 \times 10^{10} \Omega cm$  under a 100 kg/cm<sup>2</sup> loading pressure at 50% humidity and at room temperature.

The undercoat layer may be applied or coated onto a substrate by any suitable technique known in the art, such as spraying, dip coating, draw bar coating, gravure coating, silk screening, air knife coating, reverse roll coating, vacuum deposition, chemical treatment and the like. Additional vacuuming, heating, drying and the like, may be used to remove any solvent remaining after the application or coating to form the undercoat layer.

All the patents and applications referred to herein are hereby specifically, and totally incorporated herein by reference in their entirety in the instant specification.

It will be appreciated that various of the above-disclosed and other features and functions, or alternatives thereof, may be desirably combined into many other different systems or applications. Various presently unforeseen or unanticipated alternatives, modifications, variations or improvements therein may be subsequently made by those skilled in the art which are also intended to be encompassed by the following claims.

## EXAMPLES

The examples set forth herein below and are illustrative of different compositions and conditions that can be used in practicing the invention. All proportions are by weight unless otherwise indicated. It will be apparent, however, that the invention can be practiced with many types of compositions and can have many different uses in accordance with the disclosure above and as pointed out hereinafter.

### Example I

An undercoat layer dispersion was prepared as follows: a titanium oxide/phenolic resin/melamine resin dispersion was prepared by ball milling 15 grams of titanium dioxide (MT-150W, Tayca Company), 12.3 grams of the phenolic resin (VARCUM 29159, OxyChem Company, Mw of about 3,600, viscosity of about 200 cps) and 3.3 grams of the melamine resin (CYMEL 323, CYTEC) in 7.5 grams of 1-butanol, and 7.5 grams of xylene with 120 grams of 1 millimeter diameter sized  $ZrO_2$  beads for 5 days. The resulting titanium dioxide dispersion was filtered with a 20 micrometer pore size nylon cloth, and then the filtrate was measured with HORIBA CAPA 700 Particle Size Analyzer, and there was obtained a median  $TiO_2$  particle size of 50 nanometers in diameter and a  $TiO_2$  particle surface area of 30  $m^2/gram$  with reference to the above  $TiO_2$ /VARCUM/CYMEL dispersion. 0.5 grams of methyl ethyl ketone and 0.1 grams of the acid catalyst (CYC-CAT 4040, CYTEC) were added into the dispersion to obtain the coating dispersion. An aluminum drum, cleaned with detergent and rinsed with deionized water, was then coated with the above generated coating dispersion, and subsequently dried at 160° C. for 15 minutes, which resulted in an undercoat layer deposited on the aluminum and comprised of  $TiO_2$ /VARCUM/CYMEL with a weight ratio of about 63/25.9/11.1 and a thickness of 10 microns.

7

## Example II

To the above undercoat dispersion in Example I, was added 0.15 gram of 2,2'-bi(3-hydroxy-1,4-naphthoquinone) with the following chemical structure of:



A sudden color change from yellow to light red of the dispersion was observed. An aluminum drum, cleaned with detergent and rinsed with deionized water, was then coated with the above generated coating dispersion, and subsequently, dried at 160° C. for 15 minutes, which resulted in an undercoat layer deposited on the aluminum and comprised of 2,2'-bi(3-hydroxy-1,4-naphthoquinone)/TiO<sub>2</sub>/VARCUM/CYTEL with a weight ratio of about 0.63/63/25.9/11.1 and a thickness of 10 microns.

## Example III

To the above undercoat dispersion in Example I, was added 0.15 gram of 1,2-dihydroxyanthra-9,10-quinone (alizarin) with the following chemical structure of:



A sudden color change from yellow to dark red of the dispersion was observed. An aluminum drum, cleaned with detergent and rinsed with deionized water, was then coated with the above generated coating dispersion, and subsequently dried at 160° C. for 15 minutes, which resulted in an undercoat layer deposited on the aluminum and comprised of 1,2-dihydroxyanthra-9,10-quinone/TiO<sub>2</sub>/VARCUM/CYTEL with a weight ratio of about 0.63/63/25.9/11.1 and a thickness of 10 microns.

## Example IV

To the above undercoat dispersion in Example I, was added 0.15 gram of 3,4,5,6-tetrachlorocatechol with the following chemical structure of:



8

A sudden color change from yellow to dark orange of the dispersion was observed. An aluminum drum, cleaned with detergent and rinsed with deionized water, was then coated with the above generated coating dispersion, and subsequently dried at 160° C. for 15 minutes, which resulted in an undercoat layer deposited on the aluminum and comprised of 3,4,5,6-tetrachlorocatechol/TiO<sub>2</sub>/VARCUM/CYTEL with a weight ratio of about 0.63/63/25.9/11.1 and a thickness of 10 microns.

## Example V

To the above undercoat dispersion in Example I, was added 0.15 gram of 8-hydroxyquinoline with the following chemical structure of:



A sudden color change from yellow to dark orange of the dispersion was observed. An aluminum drum, cleaned with detergent and rinsed with deionized water, was then coated with the above generated coating dispersion, and subsequently dried at 160° C. for 15 minutes, which resulted in an undercoat layer deposited on the aluminum and comprised of 8-hydroxyquinoline/TiO<sub>2</sub>/VARCUM/CYTEL with a weight ratio of about 0.63/63/25.9/11.1 and a thickness of 10 microns.

## Example VI

To the above undercoat dispersion in Example I, was added 0.15 gram of 1,2,5,8-tetrahydroxyanthra-9,10-quinone (quinalizarin) with the following chemical structure of:



A sudden color change from yellow to dark red of the dispersion was observed. An aluminum drum, cleaned with detergent and rinsed with deionized water, was then coated with the above generated coating dispersion, and subsequently dried at 160° C. for 15 minutes, which resulted in an undercoat layer deposited on the aluminum and comprised of quinalizarin/TiO<sub>2</sub>/VARCUM/CYTEL with a weight ratio of about 0.63/63/25.9/11.1 and a thickness of 10 microns.

## Example VII

To the above undercoat dispersion in Example I, was added 0.15 gram of 4',5'-dibromofluorescein with the following chemical structure of:



A sudden color change from yellow to red of the dispersion was observed. An aluminum drum, cleaned with detergent and rinsed with deionized water, was then coated with the above generated coating dispersion, and subsequently dried at 160° C. for 15 minutes, which resulted in an undercoat layer deposited on the aluminum and comprised of 4',5'-dibromofluorescein/TiO<sub>2</sub>/VARCUM/CYME with a weight ratio of about 0.63/63/25.9/11.1 and a thickness of 10 microns.

#### Example VIII

To the above undercoat dispersion in Example I was added 0.15 gram of 9-phenyl-2,3,7-trihydroxy-6-fluorone with the following chemical structure of



A sudden color change from yellow to dark red of the dispersion was observed. An aluminum drum, cleaned with detergent and rinsed with deionized water, was then coated with the above generated coating dispersion, and subsequently dried at 160° C. for 15 minutes, which resulted in an undercoat layer deposited on the aluminum and comprised of 9-phenyl-2,3,7-trihydroxy-6-fluorone/TiO<sub>2</sub>/VARCUM/CYME with a weight ratio of about 0.63/63/25.9/11.1 and a thickness of 10 microns.

A chlorogallium phthalocyanine (ClGaPc) photogeneration layer dispersion was prepared as follows: 2.7 grams of ClGaPc Type B pigment was mixed with about 2.3 grams of polymeric binder VMCH (Dow Chemical) and 45 grams of n-butyl acetate. The mixture was milled in an ATTRITOR mill with about 200 grams of 1 mm Hi-Bea borosilicate glass beads for about 3 hours. The dispersion was filtered through a 20-μm nylon cloth filter, and the solid content of the dispersion was diluted to about 5 weight percent with n-butyl acetate. The ClGaPc photogeneration layer dispersion was applied on top of the above undercoat layers, respectively. The thickness of the photogeneration layer was approximately 0.2 μm. Subsequently, a 29 μm charge transport layer was coated on top of the photogeneration layer from a dispersion prepared from N,N'-diphenyl-N,N'-bis(3-methylphenyl)-1,1'-biphenyl-4,4'-diamine (5.38 grams), a film forming polymer binder PCZ 400 [poly(4,4'-dihydroxy-diphenyl-1-1-

cyclohexane, Mw=40,000)] available from Mitsubishi Gas Chemical Company, Ltd. (7.13 grams), and PTFE POLYFLON L-2 microparticle (1 gram) available from Daikin Industries dissolved/dispersed in a solvent mixture of 20 grams of tetrahydrofuran (THF) and 6.7 grams of toluene via CAVIPRO 300 nanomizer (Five Star technology, Cleveland, Ohio). The charge transport layer was dried at about 120° C. for about 40 minutes.

The above prepared photoreceptor devices were tested in a scanner set to obtain photo induced discharge curves, sequenced at one charge-erase cycle followed by one charge-expose-erase cycle, wherein the light intensity was incrementally increased with cycling to produce a series of photo induced discharge characteristic curves (PIDC) from which the photosensitivity and surface potentials at various exposure intensities were measured. Additional electrical characteristics were obtained by a series of charge-erase cycles with incrementing surface potential to generate several voltages versus charge density curves. The scanner was equipped with a scorotron set to a constant voltage charging at various surface potentials. The devices were tested at surface potentials of about 500 and about 700 volts with the exposure light intensity incrementally increased by means of regulating a series of neutral density filters. The exposure light source was a 780-nanometer light emitting diode. The aluminum drum was rotated at a speed of about 61 revolutions per minute to produce a surface speed of about 122 millimeters per second. The xerographic simulation was completed in an environmentally controlled light tight chamber at ambient conditions (about 50 percent relative humidity and about 22° C.).

Very similar photo-induced discharge curves (PIDC) were observed for all the photoreceptor devices, thus the charge transfer molecule/TiO<sub>2</sub> complexes perform very similarly to TiO<sub>2</sub> itself in undercoat layers from the point of view of PIDC.

The above photoreceptor devices were then acclimated for 24 hours before testing in J-zone (70° F./10% Room Humidity). Print tests were performed in Copeland Work centre Pro 3545 using black and white copy mode to achieve machine speed of 208 mm. After printing 200 5% area coverage documents, ghosting levels were measured against an empirical scale, where the smaller the ghosting grade level, the better the print quality. In general, a ghosting grade reduction of 1 to 2 levels was observed when charge transfer molecule/TiO<sub>2</sub> complex was applied in undercoat layer when compared to TiO<sub>2</sub> itself in undercoat layer. Therefore, incorporation of charge transfer molecule in undercoat layer significantly improves print quality such as ghosting.

What is claimed is:

1. An electrophotographic imaging member, comprising:  
a substrate;  
an undercoat layer formed on the substrate, wherein the undercoat layer comprises a complex in an amount of from about 20% to about 80% by weight of the total weight of the undercoat layer, the complex further comprising  
a charge transfer molecule, and  
TiO<sub>2</sub>; and  
at least one imaging layer formed on the undercoat layer, wherein the charge transfer molecule complexes with the TiO<sub>2</sub> to form coordination bonds and the coordination bonds provide a reduction in ghosting grade by at least one level.
2. The electrophotographic imaging member of claim 1, wherein the charge transfer molecule has one or more substructures selected from the group consisting of:

## 11



wherein Z is independently selected from the group consisting of a hydroxyl and a thio; X is independently selected from the group consisting of a hydroxyl, a thio, and a halogen atom; and Y is independently selected from the group consisting of an oxygen and a sulfur atom.

3. The electrophotographic imaging member of claim 2, wherein the charge transfer molecule is selected from the group consisting of: catechol, 4-methyl-1,2-benzenediol, 3-methyl-1,2-benzenediol, 1,2,4-benzenetriol, 1,2,3-benzenetriol, 3-fluoro-1,2-benzenediol, 3,4-dihydroxybenzonitrile, 3-methoxy-1,2-benzenediol, 5-methyl-1,2,3-benzenetriol, 2-fluoro-6-methoxyphenol, 4-chloro-1,2-benzenediol, 1,2-naphthalenediol, 2,3-naphthalenediol, 7,8-dihydroxy-2H-chromen-2-one, 6,7-dihydroxy-2H-chromen-2-one, 3,5-dichloro-1,2-benzenediol, 2-hydroxy-3,4-dimethoxybenzaldehyde, 2-chloro-4-(hydroxymethyl)-6-methoxyphenol, 2,3,4,6-tetrahydroxy-5H-benzo[a]cyclohept-5-one, 1,2,10-anthracenetiol, 1,2-dihydroxyanthra-9,10-quinone (alizarin), 3,4,5,6-tetrachlorocatechol, 7,8-dihydroxy-2-phenyl-4H-chromen-4-one, 1,2,7-trihydroxyanthra-9,10-quinone, 1,2,4-trihydroxyanthra-9,10-quinone, 3,4,5,6-tetrachloro-1,2-benzenediol, 7,8-dihydroxy-2-methyl-3-phenyl-4H-chromen-4-one, 5,6,7-trihydroxy-2-phenyl-4H-chromen-4-one, 1,2,5,8-tetrahydroxyanthra-9,10-quinone (quinalizarin), 2-(3,4-dihydroxyphenyl)-5,7-dihydroxy-4H-chromen-4-one, 3,4,6a,10-tetrahydroxy-6a,7-dihydroindeno[2,1-c]chromen-9(6H)-one, 3,7-dihydroxy-2-(4-hydroxy-3-methoxyphenyl)-4H-chromen-4-one, 2,3,7,8-tetrahydroxychromeno[5,4,3-cde]chromene-5,10-dione, 2-(3,4-dihydroxyphenyl)-3,5,7-trihydroxy-4H-chromen-4-one, nordihydroguaiaretic acid, tetrachlorocatechol, 2,4,5-trichlorophenol, 2,2'-bi(3-hydroxy-1,4-naphthoquinone), tetrahydroxy-1,4-quinone, 8-hydroxyquinoline, 4',5'-dibromo-9-phenyl-2,3,7-trihydroxy-6-fluorone, 1,2,3,4-tetrafluoro-5,8-dihydroxyanthraquinone, and mixtures thereof.

4. The electrophotographic imaging member of claim 2, wherein the charge transfer molecule is present in an amount of from about 0.1% to about 5% by weight of the total weight of the complex.

5. The electrophotographic imaging member of claim 1, wherein the TiO<sub>2</sub> is not surface treated.

6. The electrophotographic imaging member of claim 1, wherein the TiO<sub>2</sub> is surface treated with a material selected from the group consisting of: aluminum laurate, alumina, zirconia, silica, silane, methicone, dimethicone, sodium metaphosphate, and mixtures thereof.

7. The electrophotographic imaging member of claim 1, wherein thickness of the undercoat layer is from about 0.1 μm to about 30 μm.

8. A process for preparing an electrophotographic imaging member, comprising:

forming a coating mixture by blending a dispersion containing TiO<sub>2</sub> with a charge transfer molecule, thereby forming a complex including the charge transfer molecule and TiO<sub>2</sub>;

applying the coating mixture on an electrophotographic imaging member; and

## 12

causing the coating mixture to form an undercoat layer containing the complex on the electrophotographic imaging member, wherein the charge transfer molecule complexes with the TiO<sub>2</sub> to form coordination bonds and the coordination bonds provide a reduction in ghosting grade by at least one level and wherein the complex is present in an amount of from about 20% to about 80% by weight of the total weight of the undercoat layer.

9. The process of claim 8, wherein thickness of the undercoat layer is from about 0.1 μm to about 30 μm.

10. The process of claim 8, wherein the TiO<sub>2</sub> has a powder volume resistivity of from about 1×10<sup>4</sup> to about 1×10<sup>10</sup> Ωcm under a 100 kg/cm<sup>2</sup> loading pressure at 50% humidity and at room temperature.

11. A process for preparing an electrophotographic imaging member, comprising:

forming a coating mixture by dispersing a formulation containing TiO<sub>2</sub> and a charge transfer molecule, thereby forming a complex including the charge transfer molecule and TiO<sub>2</sub>, the charge transfer molecule being selected from the group consisting of 2,2'-bi(3-hydroxy-1,4-naphthoquinone), 1,2-dihydroxyanthra-9,10-quinone (alizarin), 3,4,5,6-tetrachlorocatechol, 8-hydroxyquinoline, 1,2,5,8-tetrahydroxyanthra-9,10-quinone (quinalizarin), 4',5'-dibromo-9-phenyl-2,3,7-trihydroxy-6-fluorone, and mixtures thereof;

applying the coating mixture on an electrophotographic imaging member; and

causing the coating mixture to form an undercoat layer containing the complex on the electrophotographic imaging member, wherein the charge transfer molecule complexes with the TiO<sub>2</sub> to form coordination bonds and the coordination bonds provide a reduction in ghosting grade by at least one level and wherein the complex is present in an amount of from about 20% to about 80% by weight of the total weight of the undercoat layer.

12. The process of claim 11, wherein thickness of the undercoat layer is from about 0.1 μm to about 30 μm.

13. The process of claim 11, wherein the TiO<sub>2</sub> has a powder volume resistivity of from about 1×10<sup>4</sup> to about 1×10<sup>10</sup> Ωcm under a 100 kg/cm<sup>2</sup> loading pressure at 50% humidity and at room temperature.

14. A process for preparing an electrophotographic imaging member, comprising:

treating the surface of TiO<sub>2</sub> with a charge transfer molecule, thereby forming a complex including the charge transfer molecule and TiO<sub>2</sub>;

dispersing the treated TiO<sub>2</sub>;

applying the coating mixture on an electrophotographic imaging member; and

causing the coating mixture to form an undercoat layer containing the complex on the electrophotographic imaging member, wherein the charge transfer molecule complexes with the TiO<sub>2</sub> to form coordination bonds and the coordination bonds provide a reduction in ghosting grade by at least one level and wherein the complex is present in an amount of from about 20% to about 80% by weight of the total weight of the undercoat layer.

15. The process of claim 14, wherein thickness of the undercoat layer is from about 0.1 μm to about 30 μm.

16. The process of claim 14, wherein the TiO<sub>2</sub> has a powder volume resistivity of from about 1×10<sup>4</sup> to about 1×10<sup>10</sup> Ωcm under a 100 kg/cm<sup>2</sup> loading pressure at 50% humidity and at room temperature.